

# UNITED STATES PATENT OFFICE.

DAVID E. REID, OF ROCHESTER, NEW YORK, ASSIGNOR TO EASTMAN KODAK COMPANY, OF ROCHESTER, NEW YORK, A CORPORATION OF NEW YORK.

## CELLULOSE COMPOUND.

1,116,627.

Specification of Letters Patent. Patented Nov. 10, 1914.

No Drawing.

Application filed January 31, 1914. Serial No. 815,816.

To all whom it may concern:

Be it known that I, DAVID E. REID, of Rochester, in the county of Monroe and State of New York, have invented certain new and useful Improvements in Cellulose Compounds; and I do hereby declare the following to be a full, clear, and exact description of the same.

My present invention relates to cellulosic bodies, particularly such as viscose or cellulose xanthate which have been reverted or converted into cellulose and might be termed viscid, and has for its object to adapt such material to more extended use in the arts whereby when made into pellicles or skins for film supports, for instance, the thin sheets will be rendered sufficiently tough and pliable for all practical purposes, less water absorbent than pure viscose and also less liable when dry, to cockle, thereby rendering them particularly suitable as supports for photographic and particularly moving picture film. These results are obtained by subjecting the cellulose to a treatment which I believe results in loading or impregnating it with a filling material which does not materially affect the cellulose as such, but nevertheless forms a new compound. In order that this material may be incorporated in the sheets or filaments it is desirable that it be carried into the body thereof and left there when the sheet has dried. The sheets or webs of viscose to be treated may be formed in the usual way as by flowing the liquid viscose upon a suitable surface or by projecting it through relatively small apertures and subsequently treating or reverting it by suitable chemicals or otherwise. This is one of the well known processes and produces a sheet or pellicle which is transparent, insoluble in water, but nevertheless more or less water absorbent. These sheets, pellicles or filaments are then treated while they contain moisture, (either that which is incident to their manufacture or that may be subsequently applied, as by moistening the previously dried material) preferably by removing the water and substituting therefor in the body of the cellulose the loading or filling material, and I find that this may be accomplished by treating the moist sheets to a solution composed of one or more of the alcohols or aldehydes which are miscible with water, and a filling or loading material

which is practically insoluble in water but is soluble in such alcohols or aldehydes. Among the alcohols which will answer this purpose are grain, wood and amyl, and among the aldehydes, acetic aldehyde, and 60 the ethers ethyl acetate and amyl acetate.

The quantity of the filling material employed in this solution depends somewhat upon its nature and solubility, but I find that the materials hereinafter mentioned for photographic film vary from two to fourteen per cent. of the weight of the dry reverted cellulose. The action of this solution is, I believe, to dehydrate the moistened material, and carry the loading or filling 70 material contained in the solution into the pores or interstices which contained moisture.

The character of this filling material in the solution depends to some extent upon the use for which the completed skin, pellicle or filament is adapted. As one of the particular uses for these films or skins is in the photographic art, the filling for this purpose must be of such nature that it is practically insoluble in water, will not be clouded or otherwise injuriously affected by the liquids or chemicals employed in the sensitized material subsequently applied or in the treatment to which the pellicle is subjected preparatory to being coated with the sensitized material or after, so that no chemical action will result which would affect the transparency or clearness of the pellicle, and it should be practically colorless 90 itself. On the other hand, the filling must be of such nature that it will not injuriously affect the sensitive coating (such as a gelatino argentic emulsion) either directly or when subjected to the action of the chemicals used in the photographic art or to vapors or gases, or heat and moisture. Furthermore, when used for photographic purposes this filling material should additionally consist of a high boiling point liquid or solid which is not oleaginous and is transparent when cold. I have found after considerable experimenting that I can use for the filling material for photographic use, solid crystalline bodies such as camphor, 105 triphenyl phosphate, and trinaphyl phosphate, also such high boiling point liquids as fusel oil, amyl acetate, tricresyl phosphate, benzyl acetate, benzyl benzoate, ethyl benzoate, also halogen substitution products 110

such as pentachlorethane, tetrachlorethane, and perchloroethylene. I find also for some purposes, that gums, resins and waxes, soluble in such solvents as alcohols, aldehydes and the like, and not water absorbent or soluble, and which are colorless, can well be used.

Skins or pellicles treated by subjecting them to the action of the solution for a sufficient length of time to absorb the desired amount of filling, will become, or at least the surface will become, sufficiently impregnated with the material so that even thin sheets suitable for photographic film supports are tough and pliable, and will tear with a smooth fracture instead of in the brittle and irregular manner that similar sheets formed from ordinary viscose tear or fracture. Such sheets are much less water absorbent, and when dry they lie flat, do not cockle, and will shrink and expand less than untreated sheets, all of which qualities render them desirable for use in photography, and particularly as a support for film used in taking and projecting moving pictures.

As hereinbefore stated, for some purposes the material carried into the pores need not possess all the characteristics noted which render the material especially adapted for photographic film supports, and for many purposes in the arts any filling material may be employed which is soluble in alcohols and aldehydes, etc., that are miscible with water, such filling being practically insoluble in water. The skins or pellicles may, if desired when used in photography, have their surfaces nitrated or acetylated before or after being subjected to the filling bath, then treated with a sub-stratum of such material or materials as are usually employed for the purpose, and the sensitized coating or emulsion applied in the usual or in any suitable way. In referring to the filling material as having a relatively high boiling point, I mean one having a boiling point at least as high or higher than that of water and which will remain in the cellulose sheets or filaments when subjected to temperatures approximating or below that of boiling water.

I claim as my invention:

1. In a transparent pellicle of reverted cellulose insoluble in the ordinary solvents

of converted cellulose and having incorporated in the substance thereof a filler which is non-oleaginous insoluble in water but is soluble in solvents miscible with water.

2. A transparent body comprising reverted cellulose having incorporated therein a filling material which is non-oleaginous practically insoluble in water but which is soluble in alcohols and other solvents miscible with water.

3. A transparent pellicle composed of reverted cellulose and a filling of non-oleaginous material, practically insoluble in water and soluble in alcohols and other solvents miscible with water and which does not chemically react upon or with gelatino argentic emulsion.

4. A transparent pellicle for use in photography consisting of reverted cellulose containing a filling material having the following characteristics (1) practically insoluble in water (2) soluble in alcohols and other solvents miscible with water (3) having no appreciable effect upon photographic emulsion (4) practically colorless (5) non-oleaginous and (6) incapable of chemically reacting with the chemicals used in photography in such a way as to reduce the transparency of the sheet.

5. A pellicle for use in photography composed essentially of reverted cellulose and triphenyl phosphate.

6. The method of treating reverted cellulose consisting in subjecting it while moist with water to the action of a solution embodying solvents miscible with water and a material soluble in said solvents and practically insoluble in water.

7. The method of treating pellicles of reverted cellulose for use in photography consisting in subjecting said pellicle while moist with water to the action of a solution embodying solvents miscible with water and a material practically insoluble in water.

8. The method of treating pellicles for use in photography consisting in subjecting a water damped pellicle of reverted cellulose to the action of an alcoholic solution of triphenyl phosphate.

DAVID E. REID.

Witnesses:

F. F. CHURCH,  
CHARLES E. MARTIN.